

## UNITED STATES PATENT OFFICE

2,491,774

## PENETRATING OILS

Henry E. Schulz, Winter Haven, Fla.

No Drawing. Application December 12, 1946,  
Serial No. 715,623

6 Claims. (Cl. 252—59)

**1**

This invention relates to lubricating materials and more specifically to penetrating oils containing a liquid derived from citrus fruit.

It is an object of this invention to provide novel penetrating oils containing materials derived from citrus fruit.

After oranges, lemons, grapefruit and other citrus fruit have been squeezed to extract their juice, the remaining pulp, skin and peel is processed to obtain a citrus peel oil, generally about 90% of which is a substance known as dextrolimonene or d-limonene which has a chemical formula of  $C_{10}H_{16}$ . This material is also variously known as citrene, carvene or hesperidene. Throughout the specification and claims the term "dextrolimonene" will be used to cover both the pure product  $C_{10}H_{16}$  known by all of these names and also the combination of this product with other materials usually found in citrus oils.

Dextrolimonene has been used for some time in the making of perfumes and flavoring extracts as it is a good solvent for the essences used therein. It has not, however, been used in the making of penetrating oils.

It is another object of this invention to provide novel penetrating oils containing dextrolimonene.

The present invention is based on the discovery that dextrolimonene when mixed with certain natural oils and waxes, such as liquid or solid petroleum products, castor oil and other organic fats and oils, produces a penetrating oil for loosening bolts, locks, nuts, many frozen bearings, leaf springs, etc. which is superior to any so far known. Dextrolimonene is itself not a good lubricant since it is highly volatile but when mixed with a lubricant it forms therewith a splendid penetrating oil. As a special case, dextrolimonene alone may be used as a penetrating oil where the member on which it is used (lock or bolt, for example) has some lubricant on it.

Dextrolimonene will dissolve, at ordinary temperatures, paraffin and other petroleum products and hence the lubricant can be either solid or liquid. Three examples of suitable mixtures are given below but it is to be understood that the invention is not limited to these specific examples but only as recited in the claims. In all the examples, the materials are mixed at room temperature. The examples follow:

*Example I*

|                |                    |          |
|----------------|--------------------|----------|
| Paraffin       | Per cent by weight | 0.25-23  |
| Dextrolimonene |                    | 77-99.75 |

A mixture comprising 3% paraffin and 97% dextrolimonene has been found very satisfactory.

**2***Example II*

Per cent by weight

|                              |          |
|------------------------------|----------|
| Liquid petroleum oil #30 SAE | 0.25-25  |
| Dextrolimonene               | 75-99.75 |

5 A mixture comprising 10% of #30 oil and 90% dextrolimonene has been found very satisfactory.

*Example III*

Per cent by weight

|                |          |
|----------------|----------|
| Castor oil     | 0.25-15  |
| Dextrolimonene | 85-99.75 |

In general, the amount of dextrolimonene varies from about 75% to almost, if not entirely (as in the special case mentioned above), 100%. Below 75% dextrolimonene content the mixture is not very efficient as a penetrating oil and when the dextrolimonene content closely approaches 100% the mixture is so highly volatile that it is 20 not very practical unless used immediately or kept tightly capped.

Mixtures in accordance with all of the examples given above, as well as many others, have been made and the penetrating oils formed were 25 found to be of very high quality.

What is claimed is:

1. A penetrating oil comprising a mixture of 75% to 99.75% by weight of citrus peel oil and 30 0.25% to 25% of a lubricant of the group consisting of paraffin, liquid petroleum oil and castor oil.

2. A penetrating oil comprising a mixture of 75% to 99.75% by weight of dextrolimonene and 35 0.25% to 25% of a lubricant of the group consisting of paraffin, liquid petroleum oil and castor oil.

3. A penetrating oil comprising a mixture of 77% to 99.75% by weight of dextrolimonene and 40 0.25 to 23% of paraffin.

4. A penetrating oil comprising a mixture of 75% to 99.75% by weight of dextrolimonene and 45 0.25% to 25% of a liquid petroleum oil.

5. A penetrating oil comprising a mixture of 85% to 99.75% by weight of dextrolimonene and 45 0.25% to 15% of castor oil.

6. A penetrating oil as in claim 4 in which said liquid petroleum oil is #30 SAE.

HENRY E. SCHULZ.

50

## REFERENCES CITED

The following references are of record in the file of this patent:

Mattiello: Protective and Decorative Coatings, 55 vol. I, John Wiley & Co., 1941, page 552.

Gregory: Condensed Chemical Dictionary, 3rd edition, Reinhold Publishing Company, 1942, page 250.

Bennett: Chemical Formulary, vol. 1, 1933, 60 D. Van Nostrand Company, page 363.